

## UNITED STATES PATENT OFFICE

EDWIN S. MIX, OF ROCHESTER, NEW YORK, ASSIGNOR TO HICKOK MANUFACTURING COMPANY, INC., OF ROCHESTER, NEW YORK

## LEATHER AND METHOD OF PRODUCING THE SAME

No Drawing.

Application filed July 25, 1927. Serial No. 208,413.

The present invention relates to leather and to a method of producing a novel surface on the same, and an object of the invention is to provide a novel surface on leather to prevent the leather slipping on a surface in either or both of two opposite directions and, under certain conditions, crawling or creeping on the surface.

To this and other ends, the invention consists in leather articles having a novel surface and to a process of treating the leather to produce such surface.

The invention embodies a leather of any desired form having a surface in which the major portion of the surface fibres project in either or both of two opposite directions.

In ordinary leather the surface fibres run in various directions and I have found that if the surface be combed or cut in parallel lines by a wire brush or other suitable means, the major portion of the surface fibres are released at their ends and are caused to project from the surface of the leather to provide fine projections extending in either or both of two opposite directions at a slight angle to the surface while the transverse surface fibres are cut or broken down. The rotation or movement of the brush in one direction effects the projection of a large number of fibres in that direction, and then the rotation or movement of the brush in the other direction will project other fibres in the opposite direction.

I have also found that it is possible to increase the number of surface fibres projecting in either or both of two opposite directions by a treatment of the hide during tanning to cause the major portion of the fibres to lie in parallelism. This result of paralleling the fibres may be obtained by working the hide during the tanning operations in a number of ways, such as stretching, jacking or rolling in a direction tending to influence the fibres to lie in parallelism. Other ways of rearranging the fibres in parallelism will suggest themselves to a skilled tanner depending on the kind of leather being treated. Of course, when the leather has been treated during the tanning operation to rearrange its fibres in parallelism, the combing or cutting should take place on lines parallel or sub-

stantially parallel with the rearranged fibres. The leather is capable of various uses. One use consists in employing it in garters for holding stockings and half hose in which case the surface should engage the skin or underwear of the user and the projecting fibres should extend downwardly in one direction only. This will prevent the garter slipping downwardly on the user and in fact the projecting fibres will have a tendency to cause the garter to crawl or creep upwardly on the leg. If the fibres are projected in two opposite directions the garter will have a tendency to maintain its position against shifting up or down on the leg.

What I claim as my invention and desire to secure by Letters Patent is:

1. Leather having the major portion of its fibres arranged in one general direction, and a surface combed in lines parallel with such direction.

2. The method of producing a leather surface which comprises stretching the hide in one direction during the tanning operations to cause the major portion of the fibres of the hide to arrange themselves in such direction, and combing the surface of the leather in such general direction to cut the transverse surface fibres and release the surface fibres to project in the direction of the combing.

3. Leather having the major portion of its fibres arranged in one general direction, and the transversely extending surface fibres on its flesh side cut parallel with said direction, the ends of the major portion of the surface fibres extending generally in one direction.

EDWIN S. MIX.

55

60

65

70

75

80

85

90

95

100